

# UNITED STATES PATENT OFFICE.

PHILIP M. MCKENNA, OF CONGRESS HEIGHTS, DISTRICT OF COLUMBIA.

## ALLOY STEEL.

1,389,679.

Specification of Letters Patent.

Patented Sept. 6, 1921.

No Drawing.

Application filed April 2, 1921. Serial No. 458,031.

To all whom it may concern:

Be it known that I, PHILIP M. MCKENNA, a citizen of the United States, residing at Congress Heights, in the District of Columbia, have invented certain new and useful Improvements in Alloy Steel; and I do hereby declare the following to be a full, clear, and exact description of the same.

This invention relates to the steel industry and more especially to that branch of the industry having to do with alloy steels, the objects of the invention being to produce an alloy steel possessing the qualities of toughness and resistance to breakage by shock and at the same time having the quality of red hardness, whereby it will be adapted for the manufacture of so-called "high speed" tools, etc. Heretofore steels used for lathe tools, milling cutters, hot dies, etc., have been liable to breakage under stress, as the steels heretofore available while possessing the quality of red hardness were deficient in strength.

The alloy steel of the present invention will be best understood from a general statement of the ingredients and a specific statement of the analysis of a characteristic sample. The alloy besides iron contains a large per cent. of tungsten, for example, eighteen per cent.; a smaller per cent. of chromium, say, four per cent.; carbon, say, seven-tenths of one per cent., and tantalum two and one-half per cent. The percentage of tungsten may vary from sixteen to twenty per cent.; chromium from two and one-half to five per cent.; carbon from sixty-hundredths to one and ten-hundredths per cent., and tantalum from one to three per cent. In addition to these elements, there may be present incidentally, sulfur, phosphorus, silicon, manganese, columbium, vanadium, etc., which exist as impurities in the materials used and persist in the product.

A characteristic sample of the alloy steel or chemical analysis gave the following percentages:

|          |        |
|----------|--------|
| Tungsten | 18.40% |
| Chromium | 4.18%  |
| Tantalum | 2.00%  |
| Carbon   | .78%   |

|                    |       |
|--------------------|-------|
| Sulfur             | trace |
| Phosphorus         | .009% |
| Silicon            | .40%  |
| Manganese          | .52%  |
| Columbium          | .30%  |
| Vanadium           | .28%  |
| Remainder is iron. |       |

The alloy has some remarkable advantages over ordinary red-hard steel. It hammered from the ingots without showing any cracks, while ordinary red-hard steel cracks to more or less extent while being forged. The grain, even of the cast structure, was fine in texture, and the alloy can be cast directly into milling cutters and other unforged tools, which are nonetheless strong and tough. Lathe cutting tests showed that the alloy was equal to the best high speed steel when made into tools for cutting steel at high speed. Impact tests showed that it was much more difficult to break by a sudden strain.

The method of making this steel in an electric furnace as practised at this time is to melt first all the ingredients except the tantalum, allowing for a little extra tungsten which is used to carry the tantalum as shall be described. The molten bath having been obtained, quick tests should be taken to see that the percentages of the elements in the molten alloy are such that when the tantalum (together with the small amount of tungsten which is used to carry it) is added, the content will be within the limits specified. Then a ferro alloy of tungsten and tantalum is added to the molten bath and the steel is poured after about twenty minutes.

The way in which this ferro alloy of tantalum and tungsten is prepared is to reduce together equal weights of wolframite and tantalite in an electric furnace with carbon, or other reducing agent; or the reduction may be made by the alumino thermic reaction; this results in a ferro alloy of tungsten and tantalum, the iron coming from the wolframite and tantalite mineral. The alloy resulting is purified as set forth in my U. S. Patent No. 1,208,596, processes of treating ferrotungsten. The comminuted

ferro-tungsten-tantalum, as purified by the above mentioned process, is used by throwing it into the molten bath of steel preferably in a thin sheet-iron can or container.

5 What I claim is:

1. An alloy steel of usual formula and containing 16 to 20 per cent. of tungsten,

2½ to 5 per cent. of chromium, and 1 to 3 per cent. of tantalum.

2. A mode of producing steel alloy by adding to the molten steel bath a purified alloy of tungsten, tantalum and iron.

PHILIP M. MCKENNA.